

## 1

2,998,424

**N-TRINITROETHYL AMINOTETRAZOLE**  
 Robert H. Saunders, West Chester, Pa., assignor, by  
 mesne assignments, to the United States of America  
 as represented by the Secretary of the Navy  
 No Drawing. Filed May 7, 1952, Ser. No. 286,606  
 1 Claim. (Cl. 260—308)

This invention relates to a new explosive compound, N-trinitroethyl aminotetrazole.

The new compound of the invention is a lustrous white solid which is fairly stable at room temperature. Its properties indicate that its use as an explosive is highly feasible. For example, it has a sensitivity to impact in the range of that of initiating explosives and a favorable oxygen balance.

It is an object of the invention to provide a new explosive compound, N-trinitroethyl aminotetrazole.

The compound was prepared by reacting aminotetrazole with formaldehyde and treating the resultant methylol compound with nitroform.

The invention is illustrated by the following example, but is not limited thereto.

*Example*

8.1 g. of 37% formalin solution diluted with 40 ml. of water was slowly added to an agitated aqueous suspension of 8½ g. of 5-aminotetrazole and 200 ml. of water. The agitation was continued until the solid dissolved, the solution grew cloudy, and a precipitate was finally formed. This precipitate, an intermediate methylol compound, was washed and dried. 500 mg. of the precipitate (4.35

10

15

20

25

30

## 2

m. mol) and 660 mg. of nitroform (4.35 m. mol) were mixed in a methanol solution and heated at 65° C. for several hours. This mixture was then cooled until a precipitate formed and the precipitate was washed and dried.

The compound has the following formula:



The percentage composition calculated for  $C_3H_4N_6O_6$  is 14.5 percent carbon, 1.6 percent hydrogen, 45.2 percent nitrogen and the remainder oxygen. Analysis of the compound gave 13.9 percent carbon, 1.4 percent hydrogen and 44.3 percent nitrogen. The compound has an oxygen balance of —13. Its melting point is 147° C. It gave a time of 10 minutes at 82.2° C. with the potassium iodide-starch stability test.

It is thus seen from the above that there has been provided a new compound having properties making its utility as an explosive highly feasible.

What is claimed is:

25 N-trinitroethyl aminotetrazole having the following structural formula:



No references cited.